

Feb. 16, 1965

C. M. WRIGHT

3,169,913

PREPARATION OF GEM-DINITROPARAFFINS BY ELECTROLYSIS

Filed May 10, 1961

2 Sheets-Sheet 1



FIG. 1

CHARLES M. WRIGHT  
INVENTOR.

BY  
*Ernest J. Peterson*  
AGENT

Feb. 16, 1965

C. M. WRIGHT

3,169,913

PREPARATION OF GEM-DINITROPARAFFINS BY ELECTROLYSIS

Filed May 10, 1961

2 Sheets-Sheet 2



FIG. 2

POLAROGRAPHIC *u* FROM POTASSIUM DINITROETHANE FORMED

CHARLES M. WRIGHT  
INVENTOR.

BY *Ernest G. Peterson*

AGENT

# United States Patent Office

3,169,913

Patented Feb. 16, 1965

1

3,169,913

## PREPARATION OF GEM-DINITROPARAFFINS BY ELECTROLYSIS

Charles M. Wright, Wilmington, Del., assignor to Hercules Powder Company, Wilmington, Del., a corporation of Delaware

Filed May 10, 1961, Ser. No. 109,204

14 Claims. (Cl. 204—72)

This invention relates to a method for the preparation of gem-dinitroparaffins and, more particularly, to an electrolytic method for the preparation of such compounds.

Electrolytic methods involving oxidative electrolysis of nitro compounds have not been generally utilized. This to an extent has been due to the complex reaction mechanism which takes place at the oxidative pole or anode and the uncertainty of behavior involved for obtaining end products. To a further extent, this has been due to the fact that known methods for the preparation of gem-dinitroparaffins, for example, by the electrolysis of aqueous alkaline solutions of primary nitroparaffins using a platinum or other inert anode, have been found deficient in respect to yields and current efficiencies.

Now, in accordance with the present invention, an electrolytic method has been discovered in which the reaction mechanism involving oxidative electrolysis of nitroparaffins, although difficult to define, proceeds with a certainty of behavior to yield uniform products accompanied with high yields and current efficiencies. In this method an active silver anode is electrolytically oxidized in an aqueous alkaline solution of a nitroparaffin and nitrite ion. The oxidized silver reacts with the components of the solution to form the corresponding gem-dinitroparaffin in solution and silver metal wherein the latter reprecipitates on the anode.

Thus, in the preparation of a salt of gem-dinitroparaffin by electrolysis in an electrolytic cell having a porous partition between its anode and cathode compartments, the present invention is concerned with a method which comprises passing an aqueous alkaline solution of mononitroparaffin and inorganic nitrite into the anode compartment of the cell, said solution being adjusted to a pH of from about 9 to about 13, said mononitroparaffin containing from 2 to 6 carbon atoms, and the anode being silver metal; subjecting the solution to electrolysis at from about 20 to about 75° C. wherein the silver metal is electrolytically oxidized and reacts with the components of the solution to form dinitroparaffin in solution and the silver metal is reprecipitated at the anode; and separating the dinitroparaffin thus formed from the electrolyzed solution.

In order to demonstrate the present invention, typical and preferred nitroparaffins were utilized as described in detail in the following examples.

### EXAMPLE 1

A solution consisting of 6 grams of nitroethane, 9 grams of potassium nitrite in 100 ml. of water, adjusted to pH 10 by the addition of pellets of potassium hydroxide, was prepared in a 150-ml. beaker. This was the anode solution. A silver gauze anode was inserted in the beaker. The anode was constructed by forming a flat piece of 20-mesh silver gauze, 6 x 15 cm., into a cylinder. The edges were held together with silver solder and a platinum contact was soldered to the gauze at the point where the edges of the gauze were joined. A flat-

2

bottomed, cylindrical, porous Alundum cup of 30 ml. capacity was supported in the center of the gauze anode. The bottom of the cup was approximately 1/2 inch from the bottom of the beaker. This permitted a magnetic stirrer bar to be inserted. This Alundum cup served as the cathode compartment. A cylindrical silver gauze cathode 30 sq. cm. in area was inserted in the cup. Sufficient 5% aqueous KOH was poured into the cup to raise the liquid level to that outside of the cup. The entire assembly was mounted on a magnetic stirrer, the stirrer turned on, and the anode and cathode were connected to a direct-current power source. A constant current of 4 amperes was passed for 58 minutes. The temperature in the anode compartment increased from 25° C. to 40° C. during this period. The applied potential throughout the electrolysis was between 5 and 7 volts.

At the end of the electrolysis the cathode compartment and the electrodes were removed, the anode was rinsed with a few ml. of hot water, the rinsings being added to the anode solution. The anode solution was warmed slightly (to approximately 60° C.) to ensure that all of the potassium dinitroethane formed was in solution and filtered, with the aid of vacuum, through a medium porosity glass frit. The beaker and filter frit were washed with a few ml. of hot water. This removed some silver powder that had settled to the bottom of the beaker. The filtrate was cooled in an ice bath to near 0° C. and the potassium salt of dinitroethane crystallized as yellow needles. The crystalline material was filtered off, the filtrate being saved for later analysis. The crystals were washed with acetone, dried under a gentle stream of air and weighed. The weight was 8.47 grams. The crystals were analyzed polarographically and found to contain 94% potassium dinitroethane. The filtrate from above was analyzed polarographically and found to contain 1.98 grams of potassium dinitroethane and 0.225 gram of nitroethane in solution.

The total potassium dinitroethane produced was:

$$\begin{aligned} &\text{grams} \\ &8.47 \times .94 = 7.96 \text{ (as crystals)} \\ &\text{plus } 1.98 \text{ (in solution)} \\ &\text{Total. } \underline{9.94} \end{aligned}$$

45 or

$$\frac{9.94}{158.17} = 0.0628 \text{ mole}$$

The amount of nitroethane present was 6.1 grams or

$$\frac{6.0}{75.07} = 0.0800 \text{ mole}$$

Therefore

$$\frac{0.0628}{0.0800} \times 100 = 79\%$$

converted to product.

There was 0.225 gram of nitroethane left after the electrolysis, or

$$\frac{0.225}{75} = .003 \text{ mole}$$

The moles of nitroethane consumed

$$0.0800 - 0.003 = 0.077$$

The yield was

$$\frac{0.063}{0.077} \times 100 = 82\%$$

The current efficiency was calculated as follows:

$$4 \text{ amps.} \times 58 \text{ minutes} \times 60 \text{ seconds} = 13,900 \text{ coulombs}$$

$$\frac{13,900}{96,500} = 0.144 \text{ equivalent}$$

Since it takes 2 equivalents to produce one mole of potassium dinitroethane,  $0.144/2 \times 158.2 = 11.4$  grams of potassium dinitroethane that would be produced if current efficiency was 100%.

$$\frac{9.94}{11.4} \times 100 = 87\% \text{ current efficiency}$$

### EXAMPLE 2

A solution containing 6 grams of nitroethane, 6.5 grams of sodium nitrite in 100 ml. of water, adjusted to pH 10 by the addition of sodium hydroxide was prepared in a 150-ml. beaker. This was the anode solution. The cell was set up exactly as in Example 1 using a new silver gauze anode. A constant current of 4 amperes (D.C.) was passed for 65 minutes. The temperature of the anode solution rose from 25° C. at the start of the electrolysis to 42° C. at the end. The anode solution was filtered, the anode and the filter frit washed and the washing added to the anode solution as in Example 1. In this case, the sodium dinitroethane formed was soluble so no crystallization was carried out. The anode solution was analyzed polarographically and found to contain 8.9 grams of sodium dinitroethane and 0.19 gram of nitroethane.

By analogous calculations to those shown in Example 1, 78% of original nitroethane was converted to product, the yield was 80% and the current efficiency was 80%.

### EXAMPLE 3

An electrolytic cell was assembled as follows to demonstrate the feasibility of continuous operation. The anode compartment consisted of a jacketed, medium porosity, Pyrex glass Buchner funnel, 3 inches in diameter, having a capacity of about 150 ml. The anode was a porous bed of powdered silver metal  $\frac{1}{4}$  inch deep which completely covered the filter plate or anode support of the funnel. The powdered silver metal had a particle size from 1 to 200 microns which rendered the bed porous and permitted passage of electrolyzed solution therethrough. Electrical contact for the anode was a coil of platinum wire buried in the silver powder bed. The cathode compartment was a flat-bottomed porous alundum cup of approximately 30 ml. capacity, supported so that its bottom was  $\frac{1}{2}$  inch above the bed of silver. The cathode was a cylinder of silver gauze 30 sq. cm. in area. The cell is shown schematically in FIG. 1.

An anode solution containing 30 grams of nitroethane, 45 grams of potassium nitrite, adjusted to pH 11.5 with pellets of potassium hydroxide, was prepared in 500 ml. of water. The anode compartment was filled with a portion of this solution that had been preheated to 60° C. The cathode compartment was filled with 2% KOH as the cathode solution to the same liquid level as the anode solution. A constant current of 10 amperes was passed through the cell. During the electrolysis, the anode solution continuously passed through the bed of silver metal and the filter plate. The electrolyzed anode solution was collected in a beaker or receiving flask set in an ice bath. Fresh anode solution, preheated to 60° C., was constantly added to the top of the cell to keep the liquid level constant. Temperature of the anode solution in the cell was maintained between 55° and 70° C. by cooling water passing through the jacket. The applied potential was approximately 9 volts. The anode solution passed through the cell at a rate 350 ml. per hour. The electrolysis was carried out continuously for 67 minutes, interrupted only twice, momentarily, to replace the cathode solution with fresh 2% KOH. This was necessary to prevent the build-up of very concentrated KOH in the cathode compartment.

At the end of 67 minutes, all of the fresh anode solution had been added to the cell. The electrolysis was stopped. The cathode compartment was removed and the remaining anode solution pulled through by vacuum. The electrolyzed anode solution was filtered to remove the crystalline potassium dinitroethane. The crystalline material was dried, weighed and analyzed as in Example 1. The weight obtained was 21.74 grams. This material analyzed 96% pure potassium dinitroethane by the polarograph. The filtrate was made up to 500 ml. with distilled water. There had been a loss of approximately 50 ml. in volume during the above operations. This solution was analyzed and found to contain 6.2 grams of potassium dinitroethane and 14.4 grams of nitroethane. This solution was made up to the original nitroethane, potassium nitrite concentration used for the first pass by adding 15.6 grams of nitroethane and 23 grams of potassium nitrite. The pH was adjusted to 11.5 with pellets of potassium hydroxide. The solution was recycled and electrolyzed exactly as set forth for the first pass. The time of electrolysis was 69 minutes.

The solid material crystallized from the recycled solution after drying and weighing was found to weigh 27.10 grams. This material analyzed 94% potassium dinitroethane by the polarograph. The recycle filtrate was analyzed and found to contain 5.7 grams of potassium dinitroethane and 14.0 grams of nitroethane.

Polarograms of the above two solids and of the filtrate showed no evidence of silver. The yield and current efficiency were determined as follows:

#### Yield

Total potassium dinitroethane produced:

$$\begin{array}{r} \text{grams} \\ 21.74 \times .96 = 20.9 \\ 27.10 \times .94 = 25.5 \\ \hline 5.7 \\ \hline 52.1 \end{array}$$

or

$$\frac{52.1}{158.2} = 0.33 \text{ mole}$$

Total nitroethane consumed—31.6 grams

$$\frac{31.6}{75} = 0.42 \text{ mole}$$

$$\frac{0.33}{0.42} \times 100 = 79\% \text{ overall yield}$$

#### Current efficiency

$$136 \text{ min.} \times 60 \text{ sec.} \times 10 \text{ amps.} = 71,600 \text{ coulombs}$$

$$\frac{81,600}{96,500} = 0.85 \text{ equivalent}$$

$$\frac{0.85}{2} \times 158.2 = 67 \text{ grams of potassium dinitroethane if}$$

100 current eff.

$$\frac{52.1}{67} \times 100 = 78\% \text{ current efficiency}$$

### EXAMPLE 4

An anode solution was prepared containing 7.2 grams of 1-nitropropane, 9 grams of potassium nitrite in 100 ml. of water, adjusted to pH 10 by the addition of pellets of potassium hydroxide. The cell was set up and the electrolysis carried out exactly as in Example 1. The time of electrolysis was 60 minutes at 4 amperes. The anode solution was filtered, cooled and crystalline product separated. This product was washed with acetone, air dried and placed in a dessicator. The identity of this product as the potassium salt of 1,1-dinitropropane was confirmed by C, H, N and K analyses, and by the

similarity of its UV spectrum and polarographic behavior to 1,1-dinitroethane.

|   | Calculated for Potassium 1,1-Dinitropropane (Percent) | Found (Percent) |
|---|-------------------------------------------------------|-----------------|
| C | 20.93                                                 | 21.14, 20.73    |
| H | 2.93                                                  | 2.94, 2.97      |
| O | 16.27                                                 | 15.84, 16.06    |
| K | 22.70                                                 | 23.29, 23.01    |

occur between the pH's of 13 and 9. Above pH 13, no appreciable gem-dinitro compound is formed. With pH's less than 9, the nitroparaffins are only partially converted to the aci-form. The effect of pH on the reaction is shown in FIG. 2 and Table I wherein nitroethane was used to demonstrate this effect. All runs shown in Table I were made exactly as Example 1, except that polarographic analysis was done directly on the anode solution with no separation of the crystalline potassium aci-dinitroethane.

TABLE I

| Run No.                       | g. of<br>Nitro-<br>ethane/<br>100 ml. | g. of<br>KNO <sub>2</sub> /<br>100 ml. | Initial<br>pH | Electrode           | Current      | Yield,<br>percent | Current<br>Effi-<br>ciency,<br>percent | Conver-<br>sion,<br>percent | Remarks                                                 |
|-------------------------------|---------------------------------------|----------------------------------------|---------------|---------------------|--------------|-------------------|----------------------------------------|-----------------------------|---------------------------------------------------------|
| EFFECT OF pH ON REACTION      |                                       |                                        |               |                     |              |                   |                                        |                             |                                                         |
| 1                             | 6                                     | 9                                      | 13.85         | Ag gauze—90 sq. cm. | 4 amp.—1 hr. | 25                | 27                                     | 12.5                        | pH 13.1 after 35 min.—all reaction occurred after this. |
| 2                             | 6                                     | 9                                      | 13.0          | do                  | do           | 75                | 43                                     | 40                          | pH at 30 min.—12.3.<br>pH at 60 min.—12.5.              |
| 3                             | 6                                     | 9                                      | 11.6          | do                  | do           | 90                | 58                                     | 52                          | pH at 30 min.—11.75.<br>pH at 60 min.—11.90.            |
| 4                             | 6                                     | 9                                      | 10.5          | do                  | do           | 83                | 61                                     | 55                          | pH at 30 min.—10.5.<br>pH at 60 min.—11.2.              |
| 5                             | 6                                     | 9                                      | 9.6           | do                  | do           | 85                | 77                                     | 72                          | pH at 30 min.—9.70.<br>pH at 60 min.—11.0.              |
| 6                             | 6                                     | 9                                      | 9.4           | do                  | do           | 88                | 80                                     | 75                          | pH at 60 min.—11.0.                                     |
| EFFECT OF NITRITE CONCENTRATE |                                       |                                        |               |                     |              |                   |                                        |                             |                                                         |
| 7                             | 6                                     | 9                                      | 10.0          | Ag gauze—90 sq. cm. | 4 amp.—1 hr. | 92                | 89                                     | 83                          | pH at 30 min.—9.3.<br>pH at 60 min.—12.1.               |
| 8                             | 6                                     | 13.5                                   | 10.0          | do                  | do           | 76                | 69                                     | 64                          | pH at 30 min.—9.4.<br>pH at 60 min.—12.2.               |
| 9                             | 6                                     | 18                                     | 10.0          | do                  | do           | 79                | 73                                     | 68                          | pH at 30 min.—9.6.<br>pH at 60 min.—12.4.               |

## EXAMPLE 5

Solutions were prepared and electrolysis carried out exactly as in Example 4, except that 2-nitropropane was used to demonstrate the results in using a secondary nitroparaffin and the anode solution was electrolyzed for 30 minutes at 4 amperes. The electrolyzed anode solution was placed in a separatory funnel and extracted with 50 ml. of ether. The ether layer was separated and the ether evaporated off on a steam bath under a stream of nitrogen. The residue was analyzed by infrared and found to contain 2,2-dinitropropane.

From the foregoing examples, it will be appreciated that electrolytically oxidized silver can be used to prepare the aci-salt of gem-dinitroparaffins from the corresponding mononitroparaffin and nitrite ion. The silver behaves essentially catalytically in the reaction as is most evident from Example 3 which showed no evidence of silver consumption or loss.

The reaction can be carried out either with a silver gauze anode or an anode consisting of a bed of silver metal. With the silver gauze, deterioration does occur with prolonged use but it has been found, for example, that at least 48 grams of potassium aci-1,1-dinitroethane can be produced with an anode containing 15 grams of silver. Thus, 0.14 mole of silver are "consumed" in the production of 0.30 mole of 1,1-dinitroethane. However, it should be emphasized that this is not a true silver consumption. The silver merely leaves the gauze electrode surface and settles to the bottom as a fine powder. With the anode consisting of a bed of silver powder, the process can be carried out continuously and the unreacted starting material can be recycled, as heretofore demonstrated by Example 3 and schematically shown in FIG. 1.

Also, it has been found that the desired reaction will

Furthermore, it has been determined that a molar excess of from 30 to 150% nitrite ion can be used in accordance with this invention as well as stoichiometric proportions, but that as the higher nitrite concentrations are approached, reduced yields and current efficiency result. This is shown also in Table I wherein nitroethane was used to demonstrate this effect.

Still further, concentrations of the nitroparaffins within the purview of this invention may run at least as high as 12%, and with a corresponding increase in nitrite and time of electrolysis, yields and current efficiencies comparable to those set forth for Example 1 are obtainable.

It will be noted that maximum current density was not obtained in respect to the silver bed anode since its true anode area was difficult to obtain as will be the case with powdered or particulate beds. Nevertheless, in Example 3 it was demonstrated that 10 amperes of current when passed using a bed of overall area of approximately 10 sq. in. gave a current efficiency of 78%, and for continuous operation this may be further controlled and adjusted to approach the maximum effect. When silver in powdered or particulate form is utilized as the anode bed, it should have a particle size of from about 1 to about 500 microns.

Moreover, the electrolysis of nitroparaffins in accordance with this invention should be carried out at a temperature of from about 20° to about 75° C., and preferably in a vessel jacketed for cooling since the electrolysis reaction generates heat. At temperatures in the order of 80° C. and above, undue decomposition of the gem-dinitroparaffin product formed by the electrolysis occurs.

The cathode in respect to the present invention serves the ordinary function of a cathode in an electrolytic cell. The use of an identical alkali metal for the anode and cathode solutions is merely a matter of convenience.

However, some advantage is obtained when using the same strong alkali metal for the anolyte and catholyte since the catholyte by diffusion through the porous partition tends to fortify the reactive anolyte as the electrolysis proceeds. Solutions of other electrolytes may be employed as catholytes and the cathode may be an inert metal such as platinum or it may be silver which is only active from the viewpoint of reaction when used as the anode. It is essential, however, that silver be employed as the anode since it is electrolytically oxidized silver that reacts with the components of the anode solution to form the corresponding salt of dinitroparaffin. Thus, it is quite preferable to use either potassium or sodium consistently as the alkali metal for the anolyte, catholyte and source of inorganic nitrite ion. Generally, an electric current at a density of from about 0.02 to about 0.20 ampere per square centimeter of active electrode surface will be found adequate for effecting the electrolysis in accordance with this invention. However, when utilizing gauze electrodes such as set forth for Examples 1 and 2, it is quite preferable that low current densities be used.

The mononitroparaffins which may be utilized for this reaction include primary and secondary nitroparaffins containing from 2 to 6 carbon atoms. The first member of the paraffin series, nitromethane, does not react to produce a gem-dinitro compound. Thus, the mononitroparaffins which may be utilized include nitroethane, 1-nitropropane, 1-nitrobutane, 1-nitropentane, 1-nitrohexane, 2-nitropropane, 2-nitrobutane, 2-nitro-1-propanol, 1-nitro-2-propanol and 2-nitro-1,3-propanediol, with the only known requirement being that the compound form a stable, soluble aci-salt in aqueous alkali. The products obtained from the electrolysis in accordance with this invention, when a salt of gem-dinitroparaffin, may be separated from the electrolyzed anode solution by conventional procedures. For example, the preferred method of separating the potassium salt is crystallization in a cooling bath followed by filtering. The sodium salt also may be separated in this manner but this is most effectively accomplished on very concentrated solutions. The preferred procedure for separating the 40 gem-dinitroparaffin from the salt is by acidification followed by ether extraction. However, it will be appreciated that in the utilization of a secondary nitroparaffin, the product obtained is not a salt but is the gem-dinitroparaffin itself which may be separated from the electrolyzed anode solution by extraction followed by distillation.

Although it is not intended that the invention shall be limited to any particular theory of operation, the reactions that appear to take place may be written as follows wherein nitroethane, a preferred material, is used as an example.

Cathode Reaction



Anode reaction



The oxidized silver, either as free silver ion or as an insoluble silver compound, reacts as follows:



Under the conditions, as shown in Example 3, the silver metal is precipitated on or within the anode without consumption or loss thereof and, accordingly, the silver may be considered to behave catalytically.

The gem-dinitro compounds obtainable in accordance with this invention include 1,1-dinitroethane, 1,1-dinitropropane, 1,1-dinitrobutane, 1,1-dinitropentane, 1,1-dinitrohexane, 1,1-dinitro-2-propanol, 2,2-dinitropropane, 2,2-dinitrobutane, 2,2-dinitro-1-propanol and 2,2-dinitro-1,3-propanediol.

The aforementioned compounds are valuable intermediates in chemical synthesis and more recently, particu-

ly in respect to 1,1-dinitroethane, have found considerable utility as ingredients in the preparation of rocket fuels.

The advantages of this invention are multifold in that gem-dinitroparaffins can be produced continuously by electrolysis and without separation and subsequent reoxidation of large amounts of silver such as required using known chemical reactions. With these known chemical reactions, at least 2 moles of silver must be separated and reoxidized for each mole of dinitroparaffin produced. Additionally, the electrolytic method of this invention can be conducted to give high yields of the desired products and at high current efficiencies. As the examples have demonstrated, yields of at least 79% and current efficiencies of at least 78% have been obtained.

In view of the foregoing, it will be evident that this invention may be carried out by the use of various modifications and changes without departing from its spirit and scope, with only such limitations placed thereon as are imposed by the appended claims.

What I claim and desire to protect by Letters Patent is:

1. In the preparation of gem-dinitroparaffin by electrolysis in an electrolytic cell having a porous partition between its anode and cathode compartments, the method which comprises passing an aqueous alkaline solution of mononitroparaffin and inorganic nitrite into the anode compartment of the cell, said solution being adjusted to a pH between 9 and 13, said mononitroparaffin containing from 2 to 6 carbon atoms, and the anode being silver metal; subjecting the solution to electrolysis at from about 20° to about 75° C. wherein the silver metal is electrolytically oxidized and reacts with the components of the solution to form dinitroparaffin in solution and the silver metal is reprecipitated at the anode; and separating the dinitroparaffin thus formed from the electrolyzed solution.

2. In the preparation of gem-dinitroparaffin by electrolysis in an electrolytic cell having a porous partition between its anode and cathode compartments, the method which comprises passing an aqueous solution of mononitroparaffin and alkali metal nitrite into the anode compartment of the cell, said solution being adjusted to a pH between 9 and 13 by the addition of alkali metal hydroxide and the anode being silver metal; subjecting the solution to electrolysis at from about 20° to about 75° C. wherein the silver metal is electrolytically oxidized and reacts with the components of the solution to form dinitroparaffin in solution and the silver metal is reprecipitated at the anode; and separating the dinitroparaffin thus formed from the electrolyzed solution.

3. The method of claim 2 wherein the mononitroparaffin is a primary nitroparaffin.

4. The method of claim 2 wherein the mononitroparaffin is a secondary nitroparaffin.

5. The method of claim 2 wherein the mononitroparaffin is nitroethane.

6. The method of claim 2 wherein the mononitroparaffin is 1-nitropropane.

7. The method of claim 2 wherein the mononitroparaffin is 1-nitrobutane.

8. The method of claim 2 wherein the mononitroparaffin is 2-nitropropane.

9. The method of claim 2 wherein the mononitroparaffin is 2-nitrobutane.

10. The method of claim 2 wherein the mononitroparaffin is 2-nitro-1-propanol.

11. The method of claim 2 wherein the alkali metal is potassium.

12. The method of claim 2 wherein the alkali metal is sodium.

13. The method of claim 2 wherein the anode is porous silver metal powder.

14. The method of claim 2 wherein the anode is porous silver metal powder and the electrolyzed solution is recycled after separation of dinitroparaffin for make-up of

the said aqueous solution of mononitroparaffin and alkali metal nitrite.

**References Cited by the Examiner**

**UNITED STATES PATENTS**

|           |       |               |         |
|-----------|-------|---------------|---------|
| 1,218,584 | 3/17  | Sanders       | 204—292 |
| 2,485,803 | 10/49 | Bahner        | 204—79  |
| 2,583,048 | 1/52  | Hannum et al. | 260—644 |

**OTHER REFERENCES**

Plummer et al.: *Journal of American Chemical Society*, May 20, 1954, pages 2720 and 2721.

5 WINSTON A. DOUGLAS, *Primary Examiner*.

JOSEPH REBOLD, MURRAY TILLMAN, *Examiners*.